

## UNITED STATES PATENT OFFICE

2,471,390

FLUSHING COMPOSITION FOR ENGINE  
LUBRICATING SYSTEMS

John D. Morgan, South Orange, and Russell E. Lowe, East Orange, N. J., assignors to Cities Service Oil Company, New York, N. Y., a corporation of Pennsylvania

No Drawing. Application July 8, 1946,  
Serial No. 682,157

1 Claim. (Cl. 252—171)

**1**  
This invention relates to improvements in solvent compositions, and more particularly to products of this general class for use in flushing out engine lubrication systems at more or less regular intervals.

The oil composition disclosed in Patent 2,301,918 has proven to be an excellent solvent for resins, varnishes, and other gummy residues of petroleum oil, and accordingly, much more effective than the light bodied fuel oils which are conventionally employed for flushing the crankcases of automobile engines and the like. Its action upon sludge deposits, however, leaves something to be desired. While this solvent readily dissolves the resinous matter which binds the sludge to the engine walls, and thus allows the latter to break away, it has little or no power to disperse this heavy matter. In a large majority of cases the loosened sludge is broken up by mechanical agitation in the crankcase to the point where it may be circulated with the flushing composition and ultimately drained from the engine with that liquid. Occasionally, however, sludge will be brought down in such volume that mechanical agitation does not suffice to break it up, with the result that the highly viscous matter is drawn around the oil strainer to interfere with proper oil circulation. We have observed, for example, that it is somewhat hazardous to use this composition in automobile engines which have been driven for more than 35,000 miles with only conventional kerosene oil flushing. In such instances the excessive accumulation of sludge is loosened by solvent in such volume as to give rise to considerable likelihood that the oil circulation system may be completely blocked, with the corresponding possibility that the bearings may be burned, cylinders scored, etc. before the stoppage can be cleared.

The principal object of the invention is to provide a flushing composition which is a highly effective solvent for removing oil varnishes, resins, and similar gummy deposits, and is at the same time well able to disperse sludge accumulations so that this heavy matter may flow with the solvent and ultimately be drawn from the engine in suspension in that light-bodied liquid.

It is a further object of the invention to provide a composition of the foregoing kind which has the ability to work its way into close fitting bearings, around piston rings, and into other crevices to dissolve oil residues, and which will itself lubricate those and other working parts to a degree such as will permit the engine to be

**2**  
safely run at normal idling speeds during the course of the cleaning and flushing operation.

Yet another object of the invention is to provide an inexpensive and highly efficient solvent for cleaning machine parts and other general utility purposes.

Our preferred composition for use in passenger automobiles and in other engines which are subject to the same general type of intermittent service at varying loads, is made of the following ingredients in about the proportions indicated.

|                          | Per cent<br>by volume |
|--------------------------|-----------------------|
| Ortho dichloro benzene   | 49.5                  |
| Cresylic acid            | 19                    |
| Naphtha                  | 30                    |
| E. P. agent              | 1                     |
| Magnesium wax acids soap | 0.5                   |

20 In preparing this composition we make use of a commercial grade of ortho dichloro benzene, a cresylic acid of about 97-99 per cent purity, and a high flash naphtha having a boiling range of about 163°-177° F. The extreme pressure agent serves of course to impart load carrying ability to the composition. For this purpose we prefer to use a 50 per cent sulphurized tricresyl or tributyl phosphite, in about the proportions indicated. Good results can also be gotten by 25 the addition of from 1 to 2 per cent of chlor-naphtha xanthate, chloro methyl stearate, or other well-known film strength improver. The last ingredient serves the dual purpose of acting as a detergent-dispersant, and as a neutralizer to hold the pH of the composition at a value of 30 about 8. A magnesium soap which is entirely suitable for use in this composition may be prepared as follows: Molten paraffin wax (M. P. 122-126° F.) is blown with excess air for a period of from 18 to 30 hours to carry out an oxidation reaction at a temperature of from 300-315° F. or thereabouts, to yield a mixture of wax acids together with ketones, alcohols and esters, and other partial oxidation products, and some unreacted hydrocarbons. This crude mixture, having a neutralization number of about 66 and a saponification number of around 130, is then treated with naphtha, which preferably is of predominately paraffinic character, in a ratio of 35 about 10:1 by volume for the purpose of separating out naphtha-insoluble hydroxy acids and other oxidation products. The naphtha solution may then be treated with zinc chloride (preferably of about 75% concentration) or phosphoric acid (85% concentration) or both, to precipi-

tate naphtha soluble hydroxy acids and some mutually soluble oxidation products. Upon completion of this separatory treatment the naphtha solution may be flash distilled to yield a mixture consisting principally of carboxylic wax acids together with a small proportion of ketones, esters, alcohols, possibly lactides and lactones, etc. which are suitable for reaction with magnesium oxide to yield the desired soap. In general, we prefer to carry out this latter reaction by heating the wax acids to a temperature of from 290-300° F., and by then adding the magnesium oxide at a rate such as to prevent the temperature from rising much above 315° F., thereby avoiding loss of the lighter solvent constituents of the acid mixture, and excess foaming. The soap of this reaction may contain from about 1.2 to about 3.5% by weight of magnesium.

The flash point of the preferred composition is about 160° F.—well above that of kerosene and other conventional flushing oils, and within minimum limits of standard safety specifications. It is of further note that the action of the composition upon copper is substantially nil. Thus a polished strip of this material showed no corrosion after being held in the solvent for a period of six hours at a temperature of 180° F. in a standard copper corrosion test. The extreme pressure characteristics of the solvent were tested in a standard four ball machine, the results showing a steady rise in friction with increasing load, and a maximum of 14 millimeters at 500 pounds gauge, followed by seizure. In this respect the new composition is exceptionally good, and by comparison considerably better than conventional flushing oils.

The properties which have been discussed above are indications of the suitability of the composition for use in internal combustion engines. Thus its flash point is high enough to meet safety requirements, and its E. P. properties are such as to insure adequate lubrication during the flushing operation. The solvent and detergent properties of the composition were thoroughly tested on petroleum varnish and on heavy crankcase sludge. In the first instance we prepared a number of samples of petroleum varnish by baking lubricating oil on steel test strips at a temperature of 400° F. for a period of time sufficient to form hard, resinous coatings. These test strips were then immersed in our solvent for ten minutes, at the end of which time the gummy residues were so soft as to be easily wiped off. It will be appreciated, of course, that the temperature at which this test was carried out, namely, 75° F., was much lower than that encountered at normal engine operation, and that the test period was likewise shorter than the normal flushing operation. In addition, we find that by sloshing the liquid around the test strips, in a manner somewhat comparable to that which occurs in an engine crankcase during a flushing operation, the softened varnish was completely washed away.

The action of the solvent on crankcase sludge was tested in the following way: a section of 20 mesh copper screen of one inch width, was thoroughly impregnated for one inch of its length with the heavy sludge taken from the crankcase of a delivery truck after a long period of day in and day out operation. This strip was then hung in a test tube filled with our composition for a period of thirty minutes at a temperature of 75° F. It is of particular note that the composition was not agitated, but was purposely held

in a quiescent state. At the end of that time it was observed that the screen had been stripped clean, and that the sludge was thoroughly dispersed and suspended in the liquid flushing composition.

The results of the foregoing laboratory tests have been fully confirmed in actual practice. In these practical demonstrations on both passenger cars and trucks, we have followed the conventional practice of draining off the charge of dirty oil, refilling the crankcase with a suitable volume of solvent, of then running the engine for a period of 15-20 minutes at fast idling speed, followed by a draining of the flushing composition. During the course of such an operation, the highly solvent liquid was actively circulated through the lubrication system and was flushed over the bearings, pistons, and cylinder walls to act upon any gummy oil residues that were present. In this connection it is of particular note that the composition is light-bodied and has high penetrating power so that it readily worked its way through the bearings, around piston rings and between other close-fitting parts where oil residues are normally found. At the same time the solvent was thoroughly churned up in the crankcase and sloshed over the engine walls, the crank shaft, cam shaft, and other parts, so that it might loosen any sludge clinging to their surfaces. The action of the composition on the highly viscous matter which was thus brought down, appeared to be both solvent and dispersant in character. Thus the soluble portions of the sludge were dissolved, and the insoluble portion dispersed and suspended in the liquid. It was observed that the dispersed sludge material flowed with the liquid and showed no tendency to settle out; that it readily passed through the oil strainer and lube lines, and was drawn from the crankcase with the composition at the end of the flushing operation. In no instance have we encountered a sludge which will resist dispersion by our composition and retain its viscous character so as to give rise to the possibility of strainer and oil line clogging. On the contrary, we find that this solvent may be used with entire safety in engines in which sludge has accumulated to the point where use of the prior art solvent flushing oil would be hazardous. Inspection of such engines at the conclusion of the flushing operations has shown them to be substantially free of accumulated gummy residues, as well as of sludge, and to be in the best of condition to receive a fresh charge of lubricating oil.

The preferred composition is, as we have said, especially well suited for use in flushing crankcases of passenger automobiles and light trucks, and other engines which are subjected to the general kind of service. We have found that additional solvent compositions may be prepared from the same ingredients, within the range indicated below, for meeting conditions which are peculiar to gasoline and Diesel engines of the type used in heavy trucks, busses, construction machinery, and the like.

|                          |       |
|--------------------------|-------|
| Ortho dichloro benzene   | 45-55 |
| Cresylic acid            | 15-20 |
| Naphtha                  | 25-40 |
| E. P. agent              | 1-2   |
| Magnesium wax acids soap | 0.5-1 |

In addition we find that the preferred composition, as well as others made within the foregoing range, are highly useful in the degreasing

of machine parts, cleaning tools and dies, and for a wide variety of general industrial purposes. In applications of this general kind, the extreme pressure agent and wax acids soap obviously serve no useful function and may of course be omitted with a corresponding saving in cost.

Having described our invention in its broad form and illustrated it by way of specific example, what we claim as new and useful is:

A solvent composition for flushing engine lubrication systems consisting essentially of about 50 per cent by volume of ortho dichloro benzene, about 19 per cent of cresylic acid, about 30 per cent by volume of naphtha having a boiling range of about 163° to 177° F., about 1 per cent by volume of sulphurized tributyl phosphite containing

about 50 per cent sulfur, and about 0.5 per cent by volume of magnesium soap of wax acids.

JOHN D. MORGAN.  
RUSSELL E. LOWE.

## REFERENCES CITED

The following references are of record in the file of this patent:

## UNITED STATES PATENTS

| 10 | Number    | Name                  | Date          |
|----|-----------|-----------------------|---------------|
|    | 1,169,783 | Ellis                 | Feb. 1, 1916  |
|    | 1,495,005 | Dunning               | May 20, 1924  |
|    | 1,980,043 | Ellis                 | Nov. 6, 1934  |
| 15 | 2,259,872 | Baldeschwieler et al. | Oct. 21, 1941 |
|    | 2,339,096 | Morgan                | Jan. 11, 1944 |
|    | 2,356,340 | Murphree              | Aug. 22, 1944 |